

# UNITED STATES PATENT OFFICE.

URLYN CLIFTON TAINTON, OF LONDON, AND JOHN NORMAN PRING, OF CHESTER,  
ENGLAND.

## ELECTRODEPOSITION AND EXTRACTION OF ZINC.

1,247,179.

Specification of Letters Patent.

Patented Nov. 20, 1917.

No Drawing.

Application filed November 7, 1916. Serial No. 130,101.

*To all whom it may concern:*

Be it known that we, URLYN CLIFTON TAINTON, a subject of the King of England, residing at 1 London Wall Buildings, London, England, and JOHN NORMAN PRING, D. Sc., a subject of the King of England, residing at Linden Bank, Sandbach, Chester, England, have invented certain new and useful Improvements in the Electro-  
10 deposition and Extraction of Zinc, of which the following is a specification.

This invention is for improvements in or relating to the electro-deposition and extraction of zinc, and it is a modification of  
15 the invention described in the prior United States Patent No. 1059233.

In the said patent specification a process for the electrolytic deposition of metallic zinc from its salts is described which consists in adding to a solution of the salt a  
20 large percentage of acid, and a small proportion of a colloid agent, and electrolyzing the solution with a current of high density. The process is also applicable for the extraction  
25 of zinc from its ores, and in such a case a solution of a salt of zinc is formed, such for example as zinc sulfate, which is then treated as above described.

Our researches have led to the discovery  
30 that some of the advantages obtained by the process described in the specification of the prior Patent No. 1059233 mentioned above can be secured by the process as described in such specification without the presence of  
35 any colloid. Zinc can be so deposited economically, although the deposits are deficient in smoothness and devoid of luster, matters which for many purposes are of little, if any consequence.

40 According to the present invention, therefore, the process for the electrolytic deposition of metallic zinc from its salts, the subject of the said United States Patent No. 1059233, is carried out without the presence  
45 of any colloid. The process is applicable to the production of deposits of zinc where smoothness and luster are of little or no importance.

The solution employed is preferably a  
50 saturated solution of zinc sulfate and the acid is preferably sulfuric acid.

One example of a method of carrying the present invention into effect will now be described. A solution for depositing zinc consisting of a saturated solution of zinc sul-

fate in water to which is added 16% of sulfuric acid, and containing no colloid agent is employed. If it is required to deposit the zinc on a metal article, the article is placed in the solution and connected to the 60 electrical supply as the cathode, the anode being formed of either zinc or any substance which does not go into solution, as for example, lead, lead peroxid, or manganese di-  
65 oxid.

Current is passed through the solution at a very much higher density than is usually employed in the electrolytic deposition of zinc. For example, the density may be 600 amperes per square foot. With this current density the deposits obtained were firm, and the current efficiency was 94.6%.

The process may conveniently be used for extracting zinc from its ores, in which case the zinc is dissolved with an acid to form a 75 solution of a salt of zinc, as for example zinc sulfate, which is then electrolyzed as described above, or the cyclic process described in the co-pending application Serial No. 44837 is employed, in which the solution 80 is regenerated by dividing it into two portions, treating fresh ore with one portion thereof to dissolve zinc and neutralize its acid content, and thereafter mixing the neutral solution with the remaining portion for 85 further treatment by electrolysis with a current of high density, (for example 50 to 1000 amperes per square foot), the proportion employed for treating the fresh ore preferably being such that on neutralizing 90 the acid content with fresh ore and mixing the resulting neutral solution with the remaining solution, the mixture contains from 5 to 30% of free acid.

What we claim as our invention and desire to secure by Letters Patent is:—

1. A process for the extraction of metallic zinc from a zinc-containing material which consists in forming a solution of the zinc free from any colloid agent and containing a large percentage of acid, and electrolyzing it with a current of high density.

2. A process for the extraction of metallic zinc from its salts which consists in adding to a solution of the salt free from any 100 colloid agent a large percentage of acid and electrolyzing it with a current of high density.

3. A process for the extraction of metallic zinc from zinc sulfate which consists in 110

adding to a solution of the salt free from any colloid agent a large proportion of sulfuric acid and electrolyzing the solution with a current of high density.

5 4. A continuous electrolytic process for the extraction of zinc from a zinc-bearing material which consists in forming therefrom a concentrated solution of a zinc salt free from any colloid agent and containing 10 an excess of acid, electrolyzing the solution with a current of high density, and then using the electrolyzed solution to dissolve the zinc in a fresh charge of zinc-bearing material in such a manner as to retain the 15 acid content of the solution at its original concentration.

5. A continuous electrolytic process for the extraction of zinc from a zinc-bearing material which consists in forming therefrom 20 a concentrated solution of a zinc salt free from any colloid agent and containing an excess of acid, electrolyzing the solution with a current of high density, regenerating the said solution by dividing it into two 25 portions in such proportions that, when the acid in one portion is neutralized by the addition to it of a charge of zinc-bearing material and the resulting solution separated from the residue and mixed with the other portion of the electrolyzed solution which has been retained, the acid content of 30 the final solution shall be approximately the same as that of the original solution, and

then electrolyzing the regenerated solution with a current of high density.

6. A continuous process for the electrolytic extraction of metallic zinc from a zinc-bearing material which consists in adding sufficient of the zinc-bearing material to an acid to make a neutral solution free from any colloid agent, separating the neutral solution from the residue, adding an excess of acid, electrolyzing said solution by means of a current of high density and thus removing part of the zinc, then removing the solution now strongly acid and dividing it into two portions, neutralizing one portion by a further addition of zinc-bearing material, separating the neutral solution from the residue, adding the other portion of the removed solution and electrolyzing the acid solution so formed, and thereafter repeating the regenerating and electrolyzing process as described.

In testimony whereof we have signed our names to this specification in the presence of two subscribing witnesses.

URLYN CLIFTON TAINTON  
JOHN NORMAN PRING.

Witnesses to signature of Urlyn Clifton Tainton:

T. L. BOSQUI, W. M. W. BRUNSWICK,  
CHAS. ROGERS, CONSTANT GUERARD

Witnesses to signature of J. N. Ping:

W. M. W. BRUNSWICK, CONSTANT GUERARD